

Patented Jan. 5, 1932

1,839,411

# UNITED STATES PATENT OFFICE

WILLIAM F. RICHTER, OF APOLLO, PENNSYLVANIA, ASSIGNOR TO CHEMICAL HOLDING CORPORATION, OF APOLLO, PENNSYLVANIA, A CORPORATION OF DELAWARE

## MANUFACTURE OF ARTIFICIAL SILK

No Drawing.

Application filed June 27, 1929. Serial No. 374,276.

This invention relates to the manufacture of artificial silk.

The principal object of this invention is to provide a process of producing from cellulosic raw material consisting principally of wood pulp a grade of artificial silk which is superior in quality, particularly as regards the so-called "sound" and "feel", to the artificial silk heretofore prepared from wood pulp.

Other objects and advantages of this invention will become apparent during the course of the following description.

As is well known, repeated efforts have been made to improve the quality and finish of artificial silk so that it will possess certain of the advantageous properties of natural or real silk which it does not now possess. These efforts have been successful to a marked degree but the desired goal has not as yet been reached. For example, artificial silk made from wood pulp lacks to a certain degree the softness of texture or "feel" and fiber resonance or "sound" possessed by real silk. In some instances the artificial silk is so lacking in these desirable properties that it is characterized as "harsh" and "dull".

In order to overcome the above referred to disadvantages most processes of manufacturing artificial silk from wood pulp as heretofore employed have been variously modified but such modifications have met with only partial success. It is the principal purpose of this invention to provide an efficient and at the same time a simple process of manufacturing from wood pulp artificial silk which approaches real silk in the properties of "sound" and "feel".

I have discovered that artificial silk possessing the desirable properties referred to as well as the desirable properties now possessed by artificial silk prepared from wood pulp in the conventional manner may be produced by mixing with the wood pulp prior to chemical treatment in the manufacturing process very finely divided cotton, preferably in the form of cotton dust. Cotton dust is particularly advantageous for use since it produces the desired results and is very cheap

raw material and one which is ordinarily considered to be a waste product.

In the preferred practice of my process I first mix with any suitable wood pulp, such as poplar or spruce pulp, a minor proportion of cotton dust. The actual amount of cotton dust employed may be varied to a substantial extent but I have found that a mixture of ingredients consisting of from 85 to 95 per cent. wood pulp and from 15 to 5 per cent. of cotton dust produces the best results. In commercial practice from about five to eighteen pounds of clean cotton dust is mixed with approximately one hundred pounds of sulphite pulp.

After the wood pulp and finely divided cotton have been mixed together, the mixture is then treated according to any of the conventional processes of making artificial silk. For example, the mixture may be treated according to the so-called "viscose process" in any of its modified forms. Since any of the commercial practices of preparing rayon from cellulose fiber may be employed in the manufacture of artificial silk from the raw material consisting of wood pulp and cotton dust,

or such mixture together with other cellulose fiber, it is unnecessary to specifically outline any particular manufacturing process. In the ordinary viscose process the raw material is first converted into an alkali cellulose which is drained, pressed and ground into relatively finely divided form, after which the resulting material is treated with carbon disulphide in a suitable xanthating apparatus. The viscous mass produced is then ordinarily thinned and further digested with caustic after which it is filtered and aged. The aged material is then spun into a setting bath from a suitable spinnerette. This spun material after washing, bleaching and drying treatment is finally formed into finished filaments or threads of artificial silk.

When the artificial silk is prepared according to my process it possesses a remarkable softness of texture or "feel" and also a superior "sound". In addition my experiments indicate that the silk possesses a somewhat increased dry strength although the improvement in "sound" and "feel" is the most

noticeable and important result. The exact cause of the improvement in the quality of the silk due to the use of cotton dust as described is not definitely known but it appears that the cotton dust adheres to the long fiber in the wood pulp in the beginning of the process and remains in association therewith during the process. However, regardless of the exact cause of the improved results, extensive experiments and tests clearly demonstrate that the results are obtained and are directly due to the use of the cotton dust in conjunction with the wood pulp.

While the use of cotton dust is particularly advantageous in conjunction with wood pulp a certain measure of success may be obtained by employing cotton dust in conjunction with other cellulose fibers, particularly those which are structurally similar to the wood pulp fiber. However, no improved results are noticed when the cotton dust is used in conjunction with cotton linters and therefore this procedure is not recommended.

While I have described in detail the preferred practice of my process it is to be understood that the details of procedure may be modified without departing from the spirit of the invention or the scope of the subjoined claims.

30. What I claim is:

1. In the production of viscose from wood pulp and structurally similar cellulose fibers, the step of forming alkali cellulose by treatment of a mixture of a major proportion of said pulp and a minor proportion of cotton dust, with an alkali, the cotton dust fibers being substantially shorter than those of said pulp.
2. In the production of viscose from wood pulp, the step of forming alkali cellulose by treatment of a mixture of about 95 to 85 per cent of said pulp, and about 5 to 15 per cent of cotton dust, with an alkali.
3. A process of making alkali cellulose, comprising mixing wood pulp with a minor proportion of cotton dust, and subjecting said mixture to a solution of caustic soda.
4. A raw material for use in the preparation of alkali cellulose, comprising a mixture of wood cellulose fiber and cotton dust, said wood fiber constituting the preponderant portion of said mixture and its fibers being substantially longer than those of said cotton dust.
5. A raw material for use in the preparation of alkali cellulose, comprising a mixture of about 95 to 85 per cent of wood pulp and 5 to 15 per cent of cotton dust.

In testimony whereof I affix my signature.

60 WILLIAM F. RICHTER.